

Patented Feb. 16, 1937

2,071,307

## UNITED STATES PATENT OFFICE

2,071,307

## BLEACHING

Wilhelm Hirschkind, Berkeley, Calif., assignor to  
Great Western Electro-Chemical Company, a  
corporation of California

No Drawing. Application August 11, 1936, Serial  
No. 95,430

## 5 Claims. (Cl. 8—2)

This invention relates to the bleaching of groundwood pulp, particularly of groundwood pulp suspensions.

In my Reissue Patent No. 19,470, of February 19, 1935, I have disclosed the application of hydrosulphite to the bleaching of groundwood pulp. In my application Serial No. 755,929, filed December 4, 1934, I disclosed that it was advantageous to bleach groundwood pulp with a hydrosulphite at a pH maintained substantially between 5 and 6. I have now determined that it is advantageous to bleach groundwood pulp at a high temperature (of the order of 140° F.) while maintaining the pH of the groundwood pulp between 4.5 and 6.5 and preferably between 5 and 6. I have found that as the pH approaches 4 pink shades became prevalent, while the blues enter as 7 is approached.

The advantage of operation at high temperatures will be apparent upon considering prior operations under the controlled pH condition. While high temperature treatment with a hydrosulphite gave an effective bleach, the product was quite yellow. Low temperature bleaching with a hydrosulphite, while maintaining the pH between the preferred values of 5 and 6, also gave a product which was commercially acceptable but which nevertheless included to an appreciable extent objectionable yellow shades. In carrying out the high temperature bleach operation it was also necessary to wash immediately following the bleaching operation.

It is my discovery that, if the high temperature operation be combined with the pH control, the product secured is more purely white, the objectionable yellow shades of the cold treatment or treatment without pH control being substantially entirely eliminated.

In addition, I have found that materials need not be washed immediately following the bleach operation, the objectionable compounds formed in the high temperature bleach operation, in the absence of pH control, being eliminated when pH control is exercised. Obviating the necessity of the wash eliminates the high cost of equipment for this operation.

In carrying out this invention advantage can be taken of the high temperature produced at the pulp grinders as the hydrosulphite is added to the grinder showers or to the grinder pits. Any salt of hydrosulphurous acid, as sodium, potassium or zinc hydrosulphite, can be utilized, and the hydrosulphite can be formed in any manner well known in the art. The temperature at the grinders usually runs between 100° and 212° F.,

usually about 140° F., and between 140° and 180° F. Instead of utilizing the heat at the grinders, artificial heat can be resorted to, but this is of course more expensive.

The material utilized to maintain the pH between 4.5 and 6, and preferably between 5 and 6, must be chosen with care—a material so strongly acid or alkaline that the pH at the end is carried beyond the range specified is not useful. I have successfully used as materials for maintaining the desired pH values diammonium phosphate, sodium bicarbonate, and sodium borate. The borates, bicarbonates, phosphates, sulphites, carbonates, acetates and formates of the alkali metals, including the ammonium radical, are useful, as are calcium sulphite, phosphate and borate.

The amount of the alkaline material used is quite small, being approximately one-fifth the quantity of the hydrosulphite in the case of diammonium phosphate, and about one-fourth the quantity in the case of sodium bicarbonate. Since the amount of hydrosulphite employed is relatively small, from 0.25% to 10% the amount of the salt utilized is also small, particularly when it is pointed out that 1% of the hydrosulphite usually suffices.

After the bleaching operation, the pulp is treated in whatever manner desired to finally convert it into paper.

## I claim:

1. Bleaching ground wood at a temperature between 100° and 212° F. with a hydrosulphite at a pH substantially between 4.5 and 6.5 while maintaining said pH during said bleaching by addition of an inorganic buffering salt effective to maintain said pH substantially constant.

2. A process for treatment of a mechanical wood pulp suspension comprising subjecting pulp in said suspension at a temperature of 100° to 212° F. to reduction by a salt of hydrosulphurous acid while maintaining said suspension at a pH substantially between 4.5 and 6.5 by addition of an inorganic salt effective to maintain said pulp substantially at said pH.

3. Bleaching ground wood at a temperature between 100° and 212° F. with a hydrosulphite at a pH substantially between 5 and 6 while maintaining said pH during said bleaching by addition of an inorganic buffering salt effective to maintain said pH substantially constant.

4. A process for treatment of a mechanical wood pulp suspension comprising subjecting pulp in said suspension at a temperature of 100° to 212° F. to reduction by a salt of hydrosulphurous

1120

X 1122

X 1125

X 1169

5

10

15

20

25

30

35

40

45

50

55

acid while maintaining said suspension at a pH substantially between 5 and 6 by addition of an inorganic salt effective to maintain said pulp substantially at said pH.

5 5. A process for bleaching a ground wood pulp comprising subjecting said pulp at a temperature between 100° and 212° F. to the action of a hydro-

sulphite present in an amount of about 1% of the weight of the pulp and while maintaining the pH of said pulp between 4.5 and 6.5 by addition of an inorganic salt present in amount of about 0.25% of the weight of the pulp.

5

WILHELM HIRSCHKIND.